# EUROPEAN PATENT APPLICATION

(11) **EP 1 566 218 A1**
(43) Date of publication of application: **24.08.2005**
(21) Application number: 05001017.2
(22) Date of filing: 19.01.2005
(51) Int. Cl.: B02C 4/04, B02C 4/28

(54) **Roll mill with end plates comprising a ceramic layer**

(30) Priority: 23.02.2004 JP 2004045602
(71) Applicant: INOUE MFG., INC., Kanagawa-ken (JP)
(72) Inventor: Sano, Masahiro, Isehara-shi Kanagawa-ken (JP)
(74) Representative: Klingseisen, Franz

(57) **Abstract**

A roll mill, which comprises rolls and end plates provided at both side ends of adjacent rolls, in which a material to be mixed and milled, and dispersed is put between the rolls for a milling and dispersing treatment, wherein the inclusion of abrasion powder of the end plates into the treated material can be reduced to a great extent.

As the roll for the roll mill, a ceramic roll having a ceramic layer on its surface is preferably used. The end plates provided at both side ends of a rear roll and an intermediate roll has a ceramic layer formed on a surface which is in contact with the roll surface. The ceramic layer is formed on an inner side plate, and this inner side plate is attached to a substrate. As the ceramic layer, preferred is a flame sprayed ceramic layer formed by flame spraying a ceramic material on a base material of the inner side plate made of a copper alloy.

## Description

### (1) Technical Field to which the Invention Belongs

The present invention relates to a roll mill used for a milling and dispersing treatment of materials in production steps of various products such as printing inks, cosmetics, paints, foods, medicines and electronic part materials.

### (2) Prior Art

A roll mill, for example, a triple roll mill, comprises a rear roll, an intermediate roll and a front roll adjoining one another. The roll mill is constituted so that the material to be treated by mixing and milling, and dispersing, is poured between the two rolls i.e. the rear roll and the intermediate roll, and when it passes through a gap between the rolls, it is ground and milled and transferred to the front roll, and recovered by a doctor knife adjoining to the front roll. For example, such roll mill is disclosed in JP-A-2004-25075. And, end plates are provided at both side ends of the rear roll and the intermediate roll so as to block the side spaces between the rolls so that the material poured between the rolls will not run down from the sides of the rolls.

As the material for the end plates, taking the sealing properties of the material to be treated into account and in order to make a process for rubbing with roll surfaces easy, a copper alloy or an engineering plastic such as polyacetal or nylon is usually used. Since the end plates are in slidably contact with the roll surfaces to keep the sealing properties at the time of operating the roll mill, abrasion is caused and the abrasion powder may be included in the material to be treated. The inclusion of the abrasion powder, even if the included amount is minute, brings about some problem depending on the type of product. For example, in the production step of electronic part material etc., contamination caused by the inclusion of foreign matters in the product is a big problem.

### Summary of the Invention

It is an object of the present invention to solve the problem of contamination due to such inclusion in the product by extremely reducing the abrasion amount of end plates being in slidably contact with roll surfaces in a roll mill for a milling and dispersing treatment of a material poured between the rolls.

It is also an object of the present invention to provide end plates of a roll mill which is hardly broken and has a light weight and which is obtainable economically.

The present invention provides a roll mill, which comprises rolls and end plates provided at both side ends of adjacent rolls, in which a material to be mixed and milled, and dispersed is put therebetween for a milling and dispersing treatment, wherein the surface of each of the end plates which are in slidably contact with the surfaces of the rolls is made of a ceramic layer.

Further, according to the present invention, the ceramic layer of each end plate is a flame sprayed ceramic layer formed by flame spraying a ceramic material on the surface of a main body of each end plate; or an integral ceramic layer formed by integrally forming the main body of each end plate itself by a ceramic material. These ceramic layers are preferably formed on an inner side plate which is detachable from the substrate. More preferably, as the roll of the roll mill of the present invention, a ceramic roll having a ceramic layer on its surface is used.

In the roll mill of the present invention, since the surface of each end plate which is in slidably contact with the roll surfaces is made of a ceramic layer which is excellent in abrasion resistance and heat resistance and has a high hardness, the abrasion amount can be substantially reduced as compared with conventional end plates made of a copper alloy or an engineering plastic, whereby the contamination by inclusion in the product can be prevented. By using a ceramic roll having a ceramic layer on its surface and combining the ceramic roll and the above end plates, contamination by inclusion can further be prevented.

Further, as the main body of each end plate is integrally formed by a ceramic material, an integral ceramic layer can be formed, whereby the production is made easily. Furthermore, by forming a flame sprayed ceramic layer by flame spraying a ceramic material on the surface of the main body of the end plate, cracks and chips are hardly generated, and there is less probability that the chipped pieces enter between the gap of rolls and the roll main body is damaged. In addition, when an inner side plate is detachably attached to the substrate and a ceramic layer is formed on the inner side plate, it is possible to reduce the weight as compared with an integrally formed product, and handling can be made easily at the time of washing, setting it onto the roll main body etc.; and even it is abraded due to the use for a long time, it can be recovered by re-flame spraying, such being economical.

### Brief Explanation of Drawings

Fig.1 is an explanatory view showing an example of the roll mill of the present invention.
Fig.2 is an enlarged cross-sectional view of a part of the portion of the rolls and the end plate.
Fig.3 is a perspective view showing an example of the end plate.
Fig.4 is an enlarged cross-sectional view of a part of the end plate having a flame sprayed ceramic layer.
Fig.5 is an enlarged cross-sectional view of a part of the end plate having an integral ceramic layer.

### Preferred Embodiments of the Invention

Fig.1 shows an example to which the present invention is applied, and illustrates a triple roll mill having a rear roll (1), an intermediate roll (2) and a front roll (3), and end plates (4) provided at both side ends of the rear roll (1) and the intermediate roll (2). A material to be treated poured between the rear roll (1) and the intermediate roll (2) is milled and dispersed, and transferred to the front roll (3), and scraped by a doctor knife (5). The present invention may be applied to roll mills of two rolls or four or more rolls, and the above end plates may be provided between desired rolls.

Further, each roll of the triple roll mill shown in the drawing is a ceramic roll having a ceramic layer (6) formed on the roll surface, and since this ceramic roll hardly forms abrasion powder, the present invention is most effective by using it with such ceramic roll in combination. As the case requires, the present invention may be applied to a steel roll mill constituted by a chilled roll etc.

The end plates (4) may be constructed in various shapes depending on the structure of the roll mill main body. In the example shown in Fig.3, a main body of each end plate (7) comprises an inner side plate (8) which is in slidably contact with the roll and a substrate (9) which holds the inner side plate (8); and the inner side plate (8) is detachably attached to the substrate (9) with bolts (11) in such a state that the inner side plate (8) fits in a receiving section (10) formed in the substrate (9). The substrate (9) is preferably formed from a plastic material for reduction of weight, but may be constituted by any other appropriate materials. Further, the inner side plate may be formed in the same shape as the substrate and laminated on the inner side of the substrate detachably, or the end plate main body may be integrally formed without separating it into a substrate and an inner side plate.

On the surface of the end plate (4), or at least a surface at which the end plate main body is in slidably contact with the roll surface, a ceramic layer (12) is formed. In the example shown in Fig.3, since the inner side plate (8) is in slidably contact with the roll surface, a ceramic layer (12) is formed on the surface of the inner side plate (8). The ceramic layer (12) is formed from a ceramic material which is excellent in abrasion resistance and heat resistance and has a high hardness, such as alumina (Al₂O₃) or zirconia (ZrO₂). As shown in Fig.5, when the inner side plate (8) is integrally formed from a ceramic material, an integral ceramic layer (12b) can easily be formed.

The one obtained by integrally forming it from a ceramic material as mentioned above, tends to generate cracks and chips due to the brittleness of the ceramic itself, and it sometimes becomes heavy. When there is such a concern, the base material (13) of the inner side plate (8) may be constituted by a ductile metal material such as a copper alloy, and a ceramic material as mentioned above may be flame sprayed on its surface to form a flame sprayed ceramic layer (12a) as shown in Fig.4. In this instance, when the surface of the base material is subjected to a surface treatment by sand blast or the like, and then an undercoat is applied by plasma spraying of e.g. Ni-Cr, and then the ceramic material is flame sprayed to a thickness of about 100 to 400 µm, by which the adhesion to the base material can be improved and high quality surface properties can be obtained. Here, since the flame sprayed ceramic layer can be obtained by re-flame spraying, it can be re-used without newly producing the inner side plate even when it is abraded, whereby the present invention contributes to saving of material resources and cost reduction.

### Example 1

As shown in Fig.4, a base material (13) of an inner side plate (8) was prepared by a copper alloy and an undercoat layer is formed on its surface, followed by flame spraying of alumina, to form a flame sprayed ceramic layer (12a) having a finished thickness of about 300 µm. This inner side plate (8) was attached to a plastic substrate (9) with bolts to prepare an end plate (4). When this end plate (4) was used between the rear roll and intermediate roll both made of a ceramic material as shown in Fig.1, and 3-hour operation was conducted for treatment of a material containing abrasive powder, whereupon abrasion was observed only at such a level that the trace of contact site with the roll was recognized, the abrasion amount was extremely reduced, and no contamination by inclusion of foreign matters was caused which has been problematic in the conventional production of electronic part materials. On the other hand, when similar treatment was conducted with use of an end plate made of an engineering plastic such as polyacetal or nylon, abrasion of about 1 to 2 mm was caused at the contact site, and the problem of contamination was not solved.

## Claims

1. A roll mill, which comprises rolls and end plates provided at both side ends of adjacent rolls, in which a material to be mixed and milled, and dispersed is put therebetween for a milling and dispersing treatment, wherein the surface of each of the end plates which are in slidably contact with the surfaces of the rolls is made of a ceramic layer.

2. The roll mill according to Claim 1, wherein the ceramic layer is a flame sprayed ceramic layer formed by flame spraying a ceramic material on the surface of a main body of the end plate.

3. The roll mill according to Claim 2, wherein the flame sprayed ceramic layer has a thickness of 100 to 400 µm.

4. The roll mill according to Claim 2, wherein the main body of each end plate comprises an inner side plate having a ceramic layer and a substrate holding the inner side plate, and the flame sprayed ceramic layer is formed on the inner side plate.

5. The roll mill according to Claim 4, wherein the substrate of the main body of each end plate is made of a plastic material.

6. The roll mill according to Claim 1, wherein the ceramic layer of each end plate is an integral ceramic layer formed by integrally forming the main body of each end plate itself by a ceramic material.

7. The roll mill according to Claim 5, wherein the ceramic layer of each end plate comprises an inner side plate having a ceramic layer and a substrate holding the inner side plate, and the inner side plate is formed from a ceramic material.

8. The roll mill according to Claim 7, wherein the substrate of each end plate is made of a plastic material.

9. The roll mill according to Claim 7, wherein the surface of each roll is made of a ceramic layer.
